

C. N. FORREST.  
BITUMINOUS SHEET ROOFING AND WEATHERPROOFING MATERIAL.  
APPLICATION FILED JULY 12, 1919.  
1,429,728. Patented Sept. 19, 1922.

*FIG. I.*



*FIG. II.*



WITNESSES:

*John C. Bergner*  
*James C. Bell*

INVENTOR:

*Charles N. Forrest.*

*Jolley & Paul*  
ATTORNEYS.

Patented Sept. 19, 1922.

## UNITED STATES PATENT OFFICE.

CHARLES N. FORREST, OF RAHWAY, NEW JERSEY, ASSIGNOR TO THE BARBER  
ASPHALT COMPANY, OF PHILADELPHIA, PENNSYLVANIA, A CORPORATION  
OF WEST VIRGINIA.

## BITUMINOUS SHEET ROOFING AND WEATHERPROOFING MATERIAL.

Application filed July 12, 1919. Serial No. 310,432.

To all whom it may concern:

Be it known that I, CHARLES N. FORREST, a citizen of the United States, and a resident of Rahway, in the county of Union 5 and State of New Jersey, have invented certain new and useful Improvements in Bituminous Sheet Roofing and Weatherproofing Material, whereof the following is a specification.

My invention relates to bituminous sheet roofing and weatherproofing material, and more especially to the type of material whose most highly developed form is represented by the flexible shingle with granular 15 facing now on the market. The same material is also used in continuous strips—laid overlapping like strips of tar paper—and in shorter strips slit along one edge and laid overlapping in such a way that the appearance of individual shingles is produced. In 20 all these forms, the material is used on walls as well as on roofs, and for weatherproofing purposes generally. It is my aim to produce a material of this character free, on the one 25 hand, from various practical disadvantages of such material heretofore known, and having, on the other hand, certain positive advantages of its own.

The general type of material to which I 30 refer is disclosed in the U. S. patents to H. R. Wardell, Nos. 813,336, and 851,331, granted Feb. 20 and Apr. 23, 1907, respectively. The roofing described in these 35 patents may be sufficiently characterized (for my present purpose) as comprising a base, composed of a plurality of sheets of bitumen-impregnated fabric cemented together, and bituminous coatings on both sides of said base—whose function, *inter alia*, is to 40 protect it from access of moisture or evaporation of its impregnating compound. One of these protective coatings carries a surface of granulated material or grit that forms the weather face of the material.

Another example of this general type of 45 material now on the market dispenses with the inner bituminous coat or backing.

Now so far as I am aware, all the forms 50 of such roofing material hitherto known have been open to some or all of the following disadvantages:

When used in shingle shape or "shingle strip," the material would not lie flat, but

would curl up, after being laid, in a very unsightly manner. 55

Even when it did not thus curl to an unsightly degree, the overlying layers of material did not sufficiently adhere or cling to those beneath, so that in a high wind storm they were liable to "blow up," or even blow 60 away entirely.

Besides being peculiarly liable to the disadvantages mentioned, material without the bituminous backing absorbs moisture at its 65 rear side and loses the impregnant of its fabric base by evaporation, with the result that the fabric base rots and causes the shingles to curl very pronouncedly.

I have found that by a backing of peculiar character and properties, all these disadvantages can be obviated, and the material can be given the capacity for spontaneous 70 adhesion between overlapping layers to such an extent that after laying they automatically become a practically unitary, watertight, weatherproof, fire-resistant covering. I have also discovered a method of considerably hastening and augmenting, upon occasion, the adhesion on which depends the 75 unification of the covering. How these and various other advantages can be secured through my invention will appear from the description hereinafter of the best forms and modes of execution and application at 80 present known to me, while its real scope 85 and essence will be indicated in my claims.

I have found that a thoroughly stable, strong, rugged, and satisfactory material, having the advantages of my invention in a high degree, can be produced with a base 90 comprising a single layer of fabric, instead of the plurality of layers disclosed in the Wardell patents. A suitable fabric for this purpose is a sheet of bibulous paper or felt such as is commercially known as "rag felt." 95 A continuous long strip of such paper is first saturated or impregnated with a pitch or bituminous medium—such, for example, as Trinidad or Bermudez asphalt suitably fluxed with petroleum. This may be done by immersion in a bath of the hot asphaltum at a temperature of from 300° F. to 500° F. for a sufficient length of time. After being drawn through this asphaltum bath, the felt passes between hot rolls that squeeze out the 105 excess of asphaltum, so as to leave the sur-

face of the paper "dry," and free from glossy spots or excess of asphaltum. This paper is then coated on one side with hot bituminous cement (such as steep roofing pitch or asphalt) at a temperature of 200 to 300° F. and straightway drawn under a scraper which removes all excess and levels the surface. Immediately after, while still hot, the cement-coated surface receives a liberal application of flaked or granulated slate or other suitable grit; this is pressed into the cement, so as to insure firm adhesion to the paper, by passage of the paper under a roller—or between rolls—with slight pressure. The excess of mineral is then thrown off in any suitable manner.

The foregoing steps would complete the manufacture of unbacked bituminous weatherproofing material (such as referred to above) in accordance with one of the processes in use prior to my invention,—the material being forthwith cut to length or into individual shingles and packed for shipment. While such material is protected on its grit-covered face against absorption of moisture, etc., its exposed back not only permits gradual evaporation of the constituents of the impregnating medium required to make it sufficiently fluid to enter the pores of the paper, but also permits the fabric to begin to absorb moisture at once. This is because the felt cannot be absolutely and completely saturated without being left with a glossy surface to which the subsequent bituminous cement coat would not adhere firmly enough to stay in place when the material was heated by the sun after being put in service.

My invention involves, therefore, a special "backing" of material faced as described above or in any other suitable manner. This may be formed by applying to the back of such material a high-melting, rubbery type of bituminous coating, which may be composed of oxidized petroleum; a combination of hard native asphalt or asphalts with petroleum flux; or stearine pitch. Whatever material be used, it is essential that it be water insoluble and water repellent, moderately hard, and have a melting point above 150° F. I have found that an oxidized asphaltic petroleum having a penetration of from 10° to 30° and a melting point of from 150° F. to 250° F., is a suitable bituminous coating for such use. The scale of hardness here referred to is, of course, the penetration in 5 seconds at 77° F. of a No. 2 Roberts needle loaded 100 grams, American Society for Testing Materials' standard method. It is applied hot to the roofing material before it is cut, in any convenient manner. A suitable method of application is to pass the sheet of saturated felt over a hot metal roller which is revolving in a tank of the melted bituminous material.

It is not essential that the application of the facing and the application of the backing be wholly separate and distinct operations as tacitly assumed in the foregoing description. On the contrary, their application may be combined in a single operation by drawing the impregnated strip through one single bath of material suitable for the backing as just described, so that this same material shall constitute the cement binder for the granular mineral or other gritty facing.

Inasmuch as bituminous shingles are shipped in bundles, and the back of one unit is in facial contact with the mineral covered surface of another, and the bundles are bound tightly together, it is obvious that a unique type of bituminous material must be used for the back coating, or the whole bundle of shingles will stick together before they reach the consumer. The like applies; also, to shingle strips and to rolls of continuous plain sheet material. As an extra precaution against sticking, the backs of the shingles may be dusted with finely powdered soapstone, talc, slate, or the like.

However, although sheet material faced and backed as above described will not stick to similar material under shipping conditions, nevertheless it will be found that under the natural influences and conditions of use, when the material undergoes prolonged exposure to the hot sun after laying, adhesion will occur spontaneously between the overlying back of one layer and the face of a subjacent layer to such a degree that the whole roof covering automatically becomes, in effect, one single unit,—so that the backing has a fixative function additional to its protective one. This action can be augmented and hastened by application of a suitable solvent to the back of each piece of material as it is laid or secured on the roof or other structure to be covered, so as to soften the bituminous coating somewhat and render it readily and freely adhesive at once. This may be done very expeditiously and conveniently by wiping the back with a cloth or brush that has been dipped in kerosene.

In the drawings, Fig. I represents conventionally the several layers constituting a sheet of my roofing as though removed successively at one portion.

Fig. II is a corresponding cross sectional view taken at the line II—II in Fig. I.

As herein shown, 1 represents the bituminously saturated base; 2 the bituminous cement on the weather side of the base 1, and 3 the grit thereby secured to the base; and 4 represents the fixative bituminous backing.

Having thus described my invention, I claim:

1. A flexible bituminous sheet weather-

70

80

85

90

95

100

105

110

115

120

125

130

proofing material comprising a fabric base saturated or impregnated with a bituminous medium; faced, on its weather side, with grit secured thereto with bituminous cement; and backed, on its inner side, with a water insoluble and repellent protective and fixative bituminous coating, sufficiently hard and high melting not to stick to a similar sheet under shipping conditions, but soft enough to adhere spontaneously to the facing of a subjacent similar sheet under the natural influence and conditions of use when exposed to the hot sun.

2. A flexible bituminous sheet weather-proofing material comprising a fabric base saturated or impregnated with a bituminous medium; faced, on its weather side, with grit secured thereto with bituminous cement; and backed, on its inner side, with a water insoluble and repellent bituminous coating, moderately hard and high melting so as not to stick to a similar sheet under shipping conditions, but soft enough to adhere spontaneously to the facing of a subjacent similar sheet under the natural influences and conditions of use when exposed to the hot sun, and also capable of being rendered readily and freely adhesive to the facing of a subjacent similar sheet by slight application of a solvent.

3. A flexible bituminous sheet weather-proofing material comprising a fabric base saturated or impregnated with a bituminous medium; faced, on its weather side, with grit secured thereto with bituminous cement; and backed, on its inner side, with a water insoluble and repellent protective and fixative rubbery bituminous coating, with a hardness of about 10 to 30 and a melting point of from 150° F. to 250° F., so as not to stick to a similar sheet under shipping conditions, but to adhere spontaneously to the facing of a subjacent similar sheet under the natural influences and conditions of use when exposed to the hot sun.

4. A roofing material for buildings consisting of a plurality of rectangular units applied as shingles which, under the natural influences and conditions of use when exposed to the hot sun, are automatically and spontaneously stuck together, after laying, by a bituminous coating upon the back of the individual units.

In witness whereof, I have hereunto signed my name at Philadelphia, Pennsylvania, this ninth day of July, 1919.

CHARLES N. FORREST.

Witnesses:

JAMES H. BELL,  
E. L. FULLERTON.